

Dec. 28, 1948.

H. EAVES ET AL

2,457,651

ELECTRON TUBE AND METHOD OF MAKING THE SAME

Filed March 18, 1946



Fig. 2



Fig. 1



Fig. 3

INVENTORS  
HUBERT EAVES  
PAUL D. WILLIAMS  
BY *Harold E. Eaves*

ATTORNEY

## UNITED STATES PATENT OFFICE

2,457,651

ELECTRON TUBE AND METHOD OF MAKING  
THE SAME

Hubert Eaves, San Mateo, and Paul D. Williams,  
Palo Alto, Calif., assignors to Eitel-McCullough,  
Inc., San Bruno, Calif., a corporation of California

Application March 18, 1946, Serial No. 655,068

1 Claim. (Cl. 316—19)

1

Our invention relates to electron tubes, and more particularly to improvements in electron emitter electrodes for such tubes.

Because of its advantages, the thoriated type of cathode or filament has been widely used as an emitter in electronic devices such as vacuum tubes, thoriated tungsten wire being commonly used as a filament material. It was early discovered that the electron emission property of a thoriated filament was enhanced by a process known as carburization (sometimes called carbonization). This step comprises forming a layer of metallic carbide adjacent the surface portions of the filament, this layer being tungsten carbide if the filament is of thoriated tungsten. The theory is that such carbide layer provides a store of carbon stable at the operating temperatures but available for reducing thorium to thorium.

The common method of carburization, long used in the art, is to heat the filament in an atmosphere of hydrocarbon gas such as methane or acetylene. Because the carburizing gas is a special atmosphere, this carburizing process must be performed as an independent step prior to final evacuation of the tube. The usual procedure involves complicated apparatus containing a bell jar or the like for receiving the filament, into which the carburizing gas may be admitted. The bell jar must be evacuated, after the filament has been heated in the hydrocarbon gas, to complete the carburizing step, all of which further complicates the apparatus.

Another disadvantage of the standard process is that it is practically impossible to control the degree and uniformity of carburization. When a filament is heated in a hydrocarbon atmosphere, the excess of carbon necessarily present causes the hotter portions of the filament to carburize more deeply than the colder portions. This is an accelerating phenomena because deeper carburization at a given section increases its resistance and consequently its temperature, which further increases the rate of taking carbon. That is why many filaments are lost by separation of the wire during carburization and why, even at best, filaments are weak mechanically and nonuniform in operating temperature and electron emission properties.

The broad object of our invention is to provide an improved thoriated type filament and method of making the same, whereby the above mentioned disadvantages and limitations are largely overcome.

The invention possesses other objects and features of advantage, some of which, with the fore-

2

going, will be set forth in the following description of our invention. It is to be understood that we do not limit ourselves to this disclosure of species of our invention, as we may adopt variant embodiments thereof within the scope of the claim.

Referring to the drawings:

Figure 1 is a vertical view of a tube embodying the improvements of our invention.

Figure 2 is a flow diagram of the process; and

Figure 3 is a diagrammatic view showing the filament coating step.

In terms of broad inclusion, our method of carburizing a thoriated filament comprises applying a coating of finely divided particles of carbon on the filament, and heating the filament to carburize it, the coating being applied uniformly in thickness along the filament to produce uniform carburization. Regulation of the coating thickness on a given filament serves to control the degree of carburization desired, depending upon the size of filament wire used. We prefer to apply the coating by electrodepositing carbon particles from a bath containing the particles in suspension. The coated filament is preferably sealed directly into a tube, and carburization is preferably effected by heating the filament during evacuation of the tube. This eliminates the usual precarburizing step and enables the filament to be carburized simultaneously with tube exhaust.

In greater detail and referring to the drawings, Figure 1 shows a tube embodying our improvements, the illustrated tube comprising an envelope 2 having a filament supporting stem 3 carrying an exhaust tubulation 4 and provided with a base 6 having prongs 7. The envelope encloses a filamentary cathode 8, tubular anode 9 and grid 11. Anode 9 has a cap 12 supported by bracket 13 on a lead 14 sealed to the upper portion of the envelope. Grid 11 is of the cage type comprising vertical bars terminating at a base ring 16 supported by bracket 17 on a grid lead 18 sealed to a side wall of the envelope.

Structurally speaking, the illustrated cathode 8 is of the filamentary type comprising a helix of thoriated tungsten wire welded to supporting leads 19 sealed to stem 3. As is the usual practice, stem 3 carrying the filament is sealed to the envelope at the stem flare 21. After exhaust, the tube is based and filament leads 19 are connected to a pair of base prongs 7 by suitable conductors 22.

This tube structure is merely for purposes of illustration and may be varied widely, it being

understood that our improved process is applicable to thoriated filaments of a variety of shapes and in tubes of many different designs.

Figure 2 is a flow diagram showing the major steps in our preferred process, namely, first fabricating and mounting the filament, then coating the filament with carbon, then sealing the filament in the tube, and then carburizing the filament by heating it during evacuation of the tube.

Fabrication of filament 8 by coiling a length of thoriated tungsten wire, and mounting the filament to its supporting stem 3 by welding to leads 19, is carried out in the usual manner. At this stage the filament structure is generally referred to as a "mounted filament," and ordinarily goes from this point to the "carbonizer" for treatment in a hydrocarbon gas. In our process this complicated treatment in a gaseous atmosphere is eliminated entirely, and the mounted filament is merely coated with finely divided carbon.

The carbon coating is preferably applied by electro-depositing a layer of carbon particles on the filament. Figure 3 shows a suitable coating apparatus comprising a tank 23 holding a bath 24 containing carbon particles 25 in suspension and agitated by a suitable stirring device 26. These particles are very small, preferably of microscopic size, say about one micron in diameter. The bath is so compounded as to place a predetermined charge, either positive or negative, on the particles. These principles of charged particles in the process of cataphoresis are well known. An example of a satisfactory bath composition to charge the carbon particles positively is as follows:

|                       |             |     |
|-----------------------|-------------|-----|
| Carbon powder         | grams       | 20  |
| Tannic acid (C. P.)   | do          | 2   |
| Methyl alcohol (99%)  | milliliters | 350 |
| Acetone (C. P.)       | do          | 25  |
| Perchloric acid (70%) | drops       | 4   |
| Phosphoric acid (85%) | do          | 4   |

The mounted filament is connected to the negative side of a potential source 26 and an electrode 27 say of molybdenum is connected to the positive side. A timer switch 28 is preferably included to automatically open the circuit after a predetermined interval, and means 29 is incorporated to vary the potential. During the coating step the mounted filament is dipped into the bath sufficiently to emerge filament 8 as shown in Figure 3. When the circuit is closed the positively charged carbon particles move to and deposit on the negative filament. Because of the extreme fineness of the carbon particles they build up a coating of uniform thickness along the filament. Also, the thickness of the coating may be very accurately controlled by the amount of potential and time it is applied. For example, a carbon coating .001 inch thick will be deposited in about 3 seconds at 60 volts with the bath described. By maintaining these conditions the coating thickness may be held within very close limits from filament to filament, and the thickness will not vary along the length of the filaments. The importance of this control will become evident as the description proceeds.

The mounted filament is preferably rinsed in acetone after removal from the bath. It is now ready for sealing into envelope 2. With a filament mounted on a glass stem, such as that illustrated, the sealing-in operation merely involves fusing flare 21 to the envelope wall, which is done

in accordance with usual practice. The tube is then ready for evacuation.

The tube may be exhausted by use of standard pumping equipment, the tubulation 4 being connected to a suitable vacuum pump in the usual manner. Our tube making process differs from ordinary practice in that the first part of the exhaust schedule includes a carburizing step. After the tube has been baked out and a reasonably good vacuum obtained, we heat the filament by passing current through it. The filament is heated to a temperature and for a time sufficient to convert all of the free carbon in the coating to a metallic carbide. For a thoriated tungsten filament having a carbon coating about .001 inch thick, we have found that heating to say 2100° C. for about 2 or 3 minutes is sufficient to convert the carbon to tungsten carbide. Since the tube is on the pump at this time and being continuously evacuated, any gas evolved during carburization is withdrawn from the tube.

After carburization, the filament temperature is reduced and any conventional procedure of tube exhaust followed. For example, the grid 25 and anode may be outgassed either by induction heating or by electron bombardment from the filament. Upon completion of the exhaust schedule the tube is removed from the pump by sealing off tubulation 4, and the tube is ready for basing.

Instead of effecting carburization by heating the filament in the tube, it is understood that the mounted filament may be precarburized by heating the coated filament in an oxygen free atmosphere such as an inert atmosphere of helium or argon, or by heating in a vacuum. This still has the advantage of producing a more uniformly carburized filament, but we prefer to carburize directly in the tube on the pump because of the simplicity involved. It is also understood that the filament may be heated in other ways than passing current through it, as by induction heating, but again we prefer the simpler direct heating procedure.

Many advantages are derived from our process and in addition to simplification of tube manufacture. One of these is the formation of a uniform layer or metallic carbide along the filament. This is due to the fact that the coating provides a uniform supply of carbon and limits the amount of carbon that can be taken up by any given section of the filament, regardless of how hot a given section may be. This eliminates the uneven carburization which occurs when an excess of carbon is available at a hotter section, as is the case when a filament is carburized in an atmosphere containing carbon. Limiting the amount of carbon also prevents loss of filaments during carburization, due to weak spots caused by too much carbide penetration. Furthermore, our carburized filaments in the final tubes are much stronger mechanically, and are consistent in this respect from tube to tube, as compared to filaments carburized in the usual way.

Another advantage resulting from uniform carburization along the length of a filament is that such a filament runs at a more even temperature from end to end. This means that the filament will emit electrons more uniformly along its length, which uniformity of emission improves a tube from both its operational and life standpoints.

Still another advantage of our process is that the initial application of the carbon as a coating makes it possible to control, not only the uni-

formity of carburization, but also the degree of carburization. Since the thickness of the carbon coating determines the amount of carbon available for combination as a carbide, it will be appreciated that regulation of the coating thickness will control the depth of the final carbide layer. Such control over the degree of carburization is important because it establishes the final operating temperature and emission properties of the filament. In our preferred process, the building up of the carbon layer by minute particles electrodeposited from a bath enables an operator to regulate the coating thickness within extremely close limits.

A further important advantage of our process is that the filament is carburized in the presence of substantially pure carbon, thereby eliminating the contamination of the filament by foreign substances such as present in a hydrocarbon atmosphere. Such contamination is responsible for poor and erratic emission properties which our process overcomes.

A still further advantage is that carburization may be restricted to selected portions of the filament structure, such as the filament wire only. This is easily done by masking off portions of the filament structure, as by shielding such portions with a covering material while the structure is in the bath. For example, if carbon is not desired on the center filament lead of the structure illustrated, a piece of split flexible tubing may be slipped over the center lead and removed after the coating step. Since only the coated portions are carburized when the filament is subsequently heated, it is apparent that carburization of undesired areas may be avoided. This is not possible when

carburization is carried on in a hydrocarbon atmosphere because any part of the structure which gets hot will take up carbon.

While we have described our improvements in connection with a filamentary type cathode, it is understood that the process may be used to equal advantage with thoriated cathodes of the unipotential type.

We claim:

10 The method of making an electron tube having a thoriated tungsten filament, which comprises mounting the filament on a support, immersing the mounted filament in a bath containing finely divided carbon particles in suspension, depositing by cataphoresis a coating of said particles on the filament, withdrawing the filament from the bath, enclosing the filament in the tube envelope, evacuating the envelope, and heating the filament in the envelope to carburize the filament prior to completion of evacuation.

HUBERT EAVES,  
PAUL D. WILLIAMS.

#### REFERENCES CITED

25 The following references are of record in the file of this patent:

#### UNITED STATES PATENTS

|    | Number    | Name               | Date          |
|----|-----------|--------------------|---------------|
| 30 | 1,983,668 | Jones et al. ----- | Dec. 11, 1934 |
|    | 2,410,060 | Goodale -----      | Oct. 29, 1946 |

#### FOREIGN PATENTS

|    | Number  | Country             | Date          |
|----|---------|---------------------|---------------|
| 35 | 450,788 | Great Britain ----- | July 24, 1936 |